

April 29, 1924.

1,492,349

J. R. BROWN ET AL

FLOAT FOR STEAM TRAPS AND THE LIKE AND METHOD OF MAKING SAME

Filed Feb. 8, 1922



INVENTORS  
John Rowland Brown and  
BY John C. Mullinix.

Ogallala & Fife  
ATTORNEYS

## UNITED STATES PATENT OFFICE.

JOHN ROWLAND BROWN AND JOHN C. MULLINNIX, OF CLEVELAND, OHIO, ASSIGNEES  
TO THE RELIANCE GAUGE COLUMN COMPANY, OF CLEVELAND, OHIO, A CORPORA-  
TION OF OHIO.

## FLOAT FOR STEAM TRAPS AND THE LIKE AND METHOD OF MAKING SAME.

Application filed February 8, 1922. Serial No. 535,037.

To all whom it may concern:

Be it known that we, JOHN ROWLAND BROWN and JOHN C. MULLINNIX, citizens of the United States, and residents of Cleveland, county of Cuyahoga, State of Ohio, have jointly invented a new and useful Improvement in Floats for Steam Traps and the like and Methods of Making Same, of which the following is a specification, the 10 principle of the invention being herein explained and the best mode in which we have contemplated applying that principle, so as to distinguish it from other inventions.

The present improvements relate more 15 particularly to floats composed of a hollow foundation and an external seamless metallic shell or coating formed by electro-plating such foundation instead of spinning such floats from sheet metal (usually copper) in 20 hemispheres and then lapping together and brazing the two sections at the joint. The latter has continued to be the commercial method of manufacture of such floats despite the fact that the electro-plating art 25 long ago reached a high point of development and despite the fact that inventors have from time to time suggested the possibility of employing the method of electro-plating to the making of articles of the type 30 in hand, see for example, U. S. Patent No. 256,270 to P. Barker, dated April 11, 1882, and No. 691,803 to W. F. Patton, dated January 28, 1902. It is not, however, as simple a matter as has apparently been supposed to 35 electro-deposit copper, or other metal, on such an internal hollow foundation and secure a uniform coating, particularly where the float is of the usual spherical form. There is a tendency, in other words, for the 40 deposited layer to vary in thickness so that the resulting floats will not stand up under the pressures to which they are subjected when in use, and there may even be actual 45 holes left in the deposited shell or the metal be so thin in places that holes promptly form as the result of handling or corrosion in use, thus rendering the floats permeable to a liquid.

We have discovered, however, that by the 50 use of proper means, more particularly a foundation of special construction and superficial character and the employment of certain steps all as hereinafter fully des-

cribed and particularly pointed out in the claims, we can make a float shell by electro-depositing copper or equivalent metal on an internal hollow foundation that will be superior both in the matter of strength, i. e., 55 rigidity under pressure, and durability. The annexed drawing and the following description 60 accordingly set forth in detail certain steps and means embodying the invention, such disclosed steps and means constituting, however, but one of various ways 65 in which the principle of the invention may be used.

In said annexed drawing:—

Fig. 1 is a perspective view of the improved form of hollow foundation which we employ in our method; Fig. 2 is a central section through such foundation showing as assembled therewith the spud whereby the float when completed may be connected with suitable operating mechanism; Fig. 3 is a view similar to Fig. 2 but showing the electro-deposited layer of metal as surrounding the hollow foundation or core; Fig. 4 is a view similar to Fig. 3 but on a larger scale; and Figs. 5 and 6 are sectional views illustrating modifications.

The core 1, while shown in the several figures of the drawing as of approximately spherical form, may of course take on any shape required by the exigencies of the use to which the completed float is to be put. It 85 is also a matter of indifference, so far as the present invention is concerned, whether the spud 2, or external attaching means for the float, be of the particular type herein shown and described, such spud forming 90 the subject-matter of a separate application filed by John Rowland Brown, one of the present inventors, viz, Ser. No. 505,524, filed October 5, 1921, patented Feb. 5, 1924, No. 1,482,882.

Said core 1 is preferably molded from pulp material, as for example, wood pulp or papier-mâché, and is characterized by having its exterior surface closely and more or less uniformly dotted with small rounded 95 protuberances 3. The thickness of the core shell may vary, but ordinarily such shell is not subjected to any great strains before being coated with metal and the latter is of course principally relied upon to give the 100 finished article the necessary strength.

However, if desired, the core itself may be made of such thickness as to contribute to the rigidity of such finished article to any desired degree.

5 A core of the character just described, where made of such pulp material, may be most conveniently made by employing a process such as the Drake process, this process being characterized by the employment 10 of a separable foraminous mold complementary to the exterior configuration of the article to be molded, in combination with means for injecting the pulpy fluid into such mold and expelling the fluid vehicle constituent of 15 the material so as to leave only the solid constituent of the pulp adhering to the mold. The outer surfaces of articles made by this process necessarily take the form of the foraminous mold sections due to the fact 20 that the material under the internal pressure employed is forced into and more or less through the openings in such mold sections which are ordinarily made of metal plates with closely spaced perforations constituting a fine mesh screen in effect. To 25 secure the best results in our utilization of cores made by the aforesaid process, care should be taken to have the openings in the foraminous mold section of substantially 30 uniform size and they should likewise be substantially uniformly spaced throughout the entire extent of the mold so that the resulting product, consisting of the core 1, as 35 shown in Fig. 1, will have its surface uniformly studded with tiny projections, the relative size of which is indicated by the sectional views of Figs. 2 and 3 which are drawn directly to scale for a spherical float having a diameter of 5 inches. In other 40 words, allowing for a metal shell 1/64 inch thick to be deposited on said core, the outside diameter of the latter will be, as shown 45 approximately 4 31/32 inches.

It should be stated at this point that other 45 materials, such as celluloid and even paraffine, may be molded by well known methods to form cores having an exterior surface possessing the characteristics just described, the only reason for preferring a core made 50 of pulp material being the relative simplicity attending its manufacture and corresponding decreased cost, while of course such material, if sufficiently compacted in the mold, will form a core possessing a considerable degree of frigidity and strength as 55 well as low specific gravity compared with its bulk.

Where the core is thus made of pulp material by a process such as the one described 60 above the fibers in certain cases tend to project beyond the protuberances 3 like tiny hairs and require to be smoothed down before proceeding with the electrodeposition of the metal which forms the exterior shell 65 of the float. To this end the molded core is

given a coating either of melted paraffine, sizing, or a lacquer of the kind hereinafter referred to. The surface may furthermore be polished to a certain extent after application of such coating, if desired, only a very 70 thin coating being required in order to accomplish the desired result. Thereupon, the core is ready to receive its metal coating.

First, however, the laterally projecting flange 2<sup>a</sup> of the spud 2 is cemented to the open end of the core which is depressed around the aperture therein to form an annular recess 4 of the proper size and shape to receive such flange. A solution of silicate of soda forms a satisfactory cement for use in this connection, the joint between the edge of the flange and the recess being filled flush so as to make a perfectly smooth surface and in addition such joint is sealed with a suitable lacquer, i. e., one imparting a smooth finish and at the same time capable of receiving and holding a coating of bronze or copper powder, or other material onto which the final metallic coating may be electrodeposited. Where a plain hollow 80 sphere, or like article, is desired, without any spud such as hereinbefore described being attached thereto, a curved plate 7 (Fig. 5) may be substituted for the flange 2<sup>a</sup> of such spud, thus closing the opening in the 85 core and conforming with the spherical surface thereof.

The core thus prepared and with the spud or its equivalent cemented in place, may thereupon be electroplated with copper, nickel or other suitable metal, in accordance with the well-established practice. We have found, however, that it is desirable to dust the exterior surface of such core with copper or bronze powder, rather than graphite, before placing the same in the electrolytic bath and in order to insure the sticking of such powder to the surface, the latter may be desirably entirely coated with a lacquer of the kind just referred to, instead of using the latter merely around the joint between the spud flange 2<sup>a</sup> and recess 4. A cellulose ester, such as the nitrate or acetate dissolved in one or more of the known solvents therefor constitutes a very satisfactory lacquer 100 for this purpose.

When placed in the electrolytic bath the multitude of tiny protuberances 3, despite their relatively minute size, seem to have the effect of insuring a uniformity of action over the entire surface of the shell so that the deposited metal builds up evenly everywhere instead of tending to become localized as with the case of a core having a smooth exterior or one with projections of a more pronounced character and spaced further apart. As indicated in Figs. 3 and 4, the deposited layer 5 of metal preserves to a certain extent the irregularities of the exterior surface of the core, the protuberances 115 120 125 130

3 being reproduced in the form of somewhat flattened out protuberances 6.

Where it is desired to deposit an unusually thick coat of metal, in order to make the 5 float or equivalent article of correspondingly greater strength, it may be found desirable to stop the deposition of the metallic coat after a point has been reached where the surface can be turned or ground off to 10 give a smooth effect, without intersecting the protuberances 3 of the core. Then a further deposit of metal is had directly on such smooth metallic surface. This modification is illustrated in Fig. 6, where the 15 base layer of metal 8 is shown as thus smoothed off, following which a second layer 9 has been deposited. It will be understood, of course, that no line of demarcation exists between the two layers, but as a result of 20 the smoothing operation, the final surface will be substantially smooth, and the mottled appearance that otherwise persists will be avoided.

We have found, as the result of extensive 25 tests, that a float or other article fabricated in the manner just described presents for the amount of metal required far greater strength and rigidity than can be obtained by constructing an all metal float, using the 30 same amount of metal. At the same time we are able to secure a uniformly tight, i. e., unpunctured shell even about the spud, which is in effect integrally incorporated into such shell by the direct deposition 35 thereon of metal at the same time that the body of the core is being coated. It should not be necessary to repeat that our improved process is not limited to the fabrication 40 of floats of the kind specifically referred to herein, but is applicable to the making of floats of various shapes and sizes, as well as various articles of similar character, irrespective of the particular use for which they may be intended.

45 Other forms may be employed embodying the features of our invention instead of the one here explained, change being made in the form or construction, provided the elements stated by any of the following claims 50 or the equivalent of such stated elements be employed, whether produced by our preferred method or by others embodying steps equivalent to those stated in the following claims.

55 We therefore particularly point out and distinctly claim as our invention:—

1. In a method of making a float or like article, the steps which consist in first forming a hollow core of non-metallic material, the exterior surface of said core being covered with closely spaced tiny protuberances, and then electroplating such core.

60 2. In a method of making a float or like article, the steps which consist in first moulding a hollow core of plastic material,

the exterior surface of said core being covered with closely spaced tiny protuberances, and then electroplating such core.

3. In a method of making a float or like article, the steps which consist in first moulding a hollow core of pulp material, the exterior surface of said core being covered with closely spaced tiny protuberances, and then electroplating such core. 70

4. In a method of making a float or like article, the steps which consist in first moulding a hollow core of pulp material, the exterior surface of said core being covered with closely spaced tiny protuberances, eliminating from such surface any projecting fibers, and then electroplating said core. 80

5. In a method of making a float or like article, the steps which consist in first moulding a hollow core of pulp material, the exterior surface of said core being covered with closely spaced tiny protuberances, coating such surface with a suitable lacquer, and then electroplating said core. 85

6. In a method of making a float or like article, the steps which consist in first moulding a hollow core of pulp material, the exterior surface of said core being covered with closely spaced tiny protuberances, coating such surface with a lacquer having a cellulosic base, and then electroplating 90 said core.

7. In a method of making a float or like article, the steps which consist in first moulding a hollow core of pulp material, the exterior surface of said core being covered with closely spaced tiny protuberances, coating such surface with a lacquer having a cellulosic base, thereupon dusting such lacquered surface with a metallic powder, and then electroplating said core. 100

8. In a method of making a float or like article, the steps which consist in first moulding a hollow core of pulp material, the exterior surface of said core being covered with closely spaced tiny protuberances, then electroplating such core, smoothing off the surface of the electrodeposited layer, and thereupon electrodepositing a further layer. 105

9. In a method of making a float or like article, the steps which consist in first forming a hollow core of non-metallic material, said core having an aperture at one point in its wall, cementing a curved plate over such aperture, and then electroplating the whole. 110

10. As a new article of manufacture, a float for steam traps and the like, comprising a hollow core, the exterior surface of said core being formed with closely spaced tiny protuberances, and a metallic coat electro-deposited on said core and conforming with such protuberances. 115

11. As a new article of manufacture, a float for steam traps and the like, comprising a hollow core molded from plastic material, the exterior surface of said core being 120

- formed with closely spaced tiny protuberances, and a metallic coat electrodeposited on said core and conforming with such protuberances.
- 5 12. As a new article of manufacture, a float for steam traps and the like, comprising a hollow core of molded pulp material, the exterior surface of said core being formed with closely spaced tiny protuberances, and a metallic coat electro-deposited on said core and conforming with such protuberances.
- 10 13. As a new article of manufacture, a hollow article for use as a float for steam traps and the like, comprising a hollow core, the exterior surface of said core being formed with closely spaced tiny protuberances, and a metallic coat deposited on said core and conforming with such protuberances.
- 15 14. As a new article of manufacture, a hollow article for use as a float for steam traps and the like, comprising a hollow core of plastic material, the exterior of said core being formed with closely spaced tiny protuberances, and a metallic coat deposited on said core and conforming with said protuberances.
- 20 15. As a new article of manufacture, a hollow article for use as a float for steam traps and the like, comprising a hollow core of molded pulp material, the exterior of said core being formed with closely spaced tiny protuberances, and a metallic coat deposited on said core and conforming with such protuberances.

Signed by us, this 2nd day of February, 1922.

JOHN ROWLAND BROWN.  
JOHN C. MULLINNIX.